

J. L. HAWKINS,  
INNERSOLE FOR BOOTS AND SHOES AND METHOD OF MAKING THE SAME,  
APPLICATION FILED DEC. 13, 1916.

1,348,644.

Patented Aug. 3, 1920.

*Fig. 1.*



*Fig. 2.*



*Fig. 3.*



WITNESSES

*H. M. Conine*  
*R. H. Alderson*

INVENTOR

*Jno. L. Hawkins*  
by *Reuben Palmer Remond*  
*Attns.*

# UNITED STATES PATENT OFFICE.

JOHN L. HAWKINS, OF CINCINNATI, OHIO, ASSIGNOR TO ARMSTRONG CORK COMPANY, OF PITTSBURGH, PENNSYLVANIA, A CORPORATION OF PENNSYLVANIA.

## INNERSOLE FOR BOOTS AND SHOES AND METHOD OF MAKING THE SAME.

1,348,644.

Specification of Letters Patent.

Patented Aug. 3, 1920.

Application filed December 13, 1916. Serial No. 136,637.

*To all whom it may concern:*

Be it known that I, JOHN L. HAWKINS, a citizen of the United States, residing at Cincinnati, Hamilton county, Ohio, have invented a new and useful Improvement in 5 Innersoles for Boots and Shoes and Methods of Making the Same, of which the following is a full, clear, and exact description, reference being had to the accompanying drawings, forming part of this specification, in which—

Figure 1 is a plan view, partly broken away, of one form of inner sole embodying my invention.

15 Fig. 2 is a transverse section through a portion of a boot or shoe embodying one form of my improved inner sole, and

Fig. 3 is a view similar to Fig. 2, but showing a modification.

20 My invention is designed to provide an improved inner sole, for leather boots and shoes, which will be substantially waterproof and non-absorbent, and which will possess various other qualities which are desirable in inner soles.

In accordance with my invention I form an inner sole of a composition consisting mainly of granulated or comminuted cork and linseed oil, or their equivalents. This 30 composition is rolled out into sheets between two layers of canvas, which are largely rolled into and embedded in the composition. The inner soles are cut to the usual shape from these sheets.

35 The numeral 2 designates the body portion of one of my improved inner soles, and 3 the canvas sheets between which the composition is rolled. 4 designates the usual flange or welt rib on the under side of the 40 inner sole, and which is used in the welt or Goodyear type of shoes indicated in Fig. 2, for the purpose of securing thereto the welts 5 to which the outer sole 6 is sewed. Inasmuch as the composition of which my im-

proved insole is composed is not of sufficient strength or body to permit this flange or rib to be formed integrally therefrom, it is necessary to form it as a separate piece. It may consist of any suitable strip, such 50 as shown in Fig. 2, secured by stitching, as indicated, to the inner sole, and having fitted over it a fabric covering which also preferably covers the entire lower surface of the inner sole, as also shown in Fig. 2.

55 In this manner I am able to use my inven-

tion in the manufacture of inner soles for shoes of this type and in which it is necessary that the sole shall have the rib on the underside. 7 designates the usual filling between the outer and inner soles.

60

Fig. 3 shows one of my improved inner soles applied to a straight sewed (McKay style) shoe.

The composition which may be employed in the formation of my improved inner sole 65 will generally consist in the main of comminuted or granulated cork and boiled linseed oil. As a partial or entire substitute for cork may be used wood flour and as a partial or entire substitute for linseed oil 70 may be used any other drying or semi-drying oil. Coloring pigments will be added as required. An excellent specific formula for the purpose may be made as follows:— seventy-five pounds linseed oil (prepared 75 and treated so as to form what is known in factory practice as cement); and one hundred pounds granulated cork.

This material is not only substantially waterproof and non-absorbent, but it possesses 80 the necessary resiliency, is practically non-expansible and non-contractible, thereby preserving its shape. It is also flexible and durable, has a good body, and its use largely prevents squeaking in boots or shoes. 85

Its substantially waterproof or water resistant and non-absorbent qualities are, however, the most important.

I may also provide the upper surface of the inner sole with a varnished coating, 90 which may be made to closely imitate leather in color and texture. When this is done, the leather sock lining which is frequently fitted into a shoe over the inner sole to give it a more finished appearance may be omitted. 95 Any suitable varnish having the desired color pigment added thereto may be employed.

I claim:

1. As a new article of manufacture, an 100 inner sole for shoes consisting of a layer of cork composition having woven fabric united to the upper and lower faces of the cork composition by pressure, portions of the intermediate cork composition being 105 pressed into and partially impregnating the fabric layers, substantially as described.

2. As a new article of manufacture, an inner sole for shoes cut from a sheet of comminuted cork composition rolled with up- 110

per and lower layers of woven fabric united with the comminuted cork composition layer by the pressure of forming the sheet, portions of the intermediate composition being forced into the said fabric layers, one of the fabric layers having an external coating, substantially as described.

3. As a new article of manufacture, an insole for shoes consisting of upper and lower layers of fabric, and an intermediate filling composed mainly of comminuted cork and linseed oil in the proportions of about seventy-five pounds of linseed oil prepared and treated so as to form what is known in factory practice as cement, and one hundred pounds cork; substantially as described.

4. As a new article of manufacture, an inner sole for shoes cut from a compressed sheet, comprising an intermediate layer of comminuted cork composition having top and bottom layers of woven fabric united with an intermediate cork layer in the compression of the sheet so as to be partially impregnated therewith, substantially as described.

5. The method of making soles for shoes,

consisting in simultaneously feeding between compressing rollers upper and lower layers of woven fabric and an intermediate layer of comminuted cork composition, firmly uniting the layers as they pass between the compressing rollers by causing the cork composition to partially impregnate the fabric, and cutting insoles from the sheets thus produced, substantially as described.

6. As a new article of manufacture, an innersole for shoes cut from a sheet of comminuted cork composition rolled between upper and lower layers of woven fabric united therewith by the pressure of forming the sheet, portions of the intermediate composition being forced into said fabric layers, one of the fabric layers having a leather imitation coating applied thereto, substantially as described.

In testimony whereof, I have hereunto set my hand.

JOHN L. HAWKINS.

Witnesses:

E. J. HEINERBUCH,  
LIDA KELLER.